

Jan. 25, 1944.

M. SKOLNIK

2,340,209

BURIAL VAULT AND METHOD OF MAKING SAME

Filed July 30, 1942



INVENTOR  
Max Skolnik  
BY  
Evans & McCoy  
ATTORNEYS

## UNITED STATES PATENT OFFICE

2,340,209

BURIAL VAULT AND METHOD OF MAKING  
SAME

Max Skolnik, Chicago, Ill.

Application July 30, 1942, Serial No. 452,830

15 Claims. (Cl. 27—3)

This invention relates to burial vaults and to a method of making the same. Burial vaults have heretofore been made either of steel or concrete. Concrete vaults, even though reinforced, are objectionable because of their porosity and great weight. Steel vaults are now difficult to obtain and are undesirable for the reason that they are subject to electrolysis and chemical deterioration.

It is an object of the present invention to provide lightweight burial vaults which are impervious to moisture and not appreciably affected by water, and which may be relatively inexpensively produced.

It is another object to provide burial vaults that are relatively strong, lightweight, unaffected by water and which are composed of a readily available plastic material.

It is another object to provide a method of making burial vaults from plastic material comprising magnesium oxychloride cement, which vaults are suitable for low cost mass production and which do not require the use of a large number of molds.

It is a further object to provide relatively lightweight, low cost burial vaults consisting essentially of magnesium oxychloride cement reinforced by fibrous material, which vaults have a desirable appearance and are substantially unaffected by moisture.

Other objects will be apparent from the following detail description of the present invention, which is illustrated by the accompanying drawing, in which:

Figure 1 is a perspective view of a shapable composite sheet having a plurality of plies of fibrous material, each coated with an adherent layer of plastic, puttylike magnesium oxychloride cement;

Fig. 2 is a perspective view of the composite sheet shown in Fig. 1 and of a form for forming the central portion of a vault, with the composite sheet bent about the form in accordance with the process embodying the present invention;

Fig. 3 is a perspective view of a generally U-shaped reinforcing strip of angle-shaped cross section for strengthening the bond between the ends and the central member of the vaults embodying the present invention;

Fig. 4 is a perspective view of a completed vault embodying the present invention;

Fig. 5 is a sectional view taken on the line 5—5 of Fig. 4;

Fig. 6 is a sectional view through a corner por-

tion of the vaults taken on the line 6—6 of Fig. 5; and

Fig. 7 is an enlarged sectional view through a portion of the wall of a burial vault embodying the present invention and showing the construction thereof.

In my copending application entitled, "Casket and method of making same," Serial No. 452,831, filed July 30, 1942, I have set forth the method of making a readily deformable and moldable composite sheet material which can be shaped in the desired form and hardened rapidly to produce strong and durable articles consisting essentially of magnesium oxychloride cement reinforced by fabric. As there described, sheets consisting essentially of fibrous material are wetted with magnesium chloride solution, preferably of about 15 to 35 degrees Baumé, and after the excess is removed by squeezing or otherwise the sheets are coated with magnesium oxychloride cement paste, preferably of creamy consistency. A plurality of sheets thus coated are then preferably superimposed on each other and the magnesium oxychloride cement in the mass allowed to set up until it attains the puttylike state where it can be readily molded without adhering to the mold members.

The fabric material used for the plies is preferably of the woven type and that used for the inner plies 2 and 3 is preferably burlap. The material used for the outer ply 4 nearest the outer surface of the vault is preferably of a relatively finer woven material, such for example as muslin, in order to permit the formation of a smoother, more metallic outer surface coating.

In the preferred method of preparing the readily moldable composite sheet material 1, the superimposed plies having the magnesium oxychloride cement in substantially creamy consistency are incorporated in a heating zone having a relatively high humidity and an elevated temperature, e. g., one of the order of 100 to 135° F., for a short period to accelerate the reaction between the constituents of the cement composition. The composite material is removed from the heating zone before setting of the cement composition has progressed substantially beyond the stiff puttylike state. With the magnesium chloride in the relatively stiff puttylike state, the composite sheet may be readily cut and formed to any desired shape.

The burial vaults embodying the present invention are preferably of the air-sealing type with a boxlike cover portion 6 and a cooperating

bottom portion 7, upon which the edges of the cover portion are adapted to rest. The cover portion 6 has a central portion, preferably of arched shape, with a U-shaped transverse cross section and with two opposed, integrally formed sides 8 gradually merging together in a dome. The ends 10 are fastened to the arch-shaped central member and form a unitary boxlike structure. The upper periphery of the end portions 10, including the side edges thereof, are preferably bonded to the entire adjacent edge portions of the central member with a layer of hardened plastic material. Suitable reinforcing means, such as a generally U-shaped reinforcing member 11 having an angular cross section is preferably applied over the inner surface of the ends 10 and of the central member in the region of their juncture.

The reinforcing strips 11 may be of hardened magnesium oxychloride cement composition containing one or more layers of fibrous material, such as burlap, and may be formed from plastic sheet material, such as that shown in Fig. 1. One side edge 12 of the angular reinforcing strip 11 is adhered to the edge portions of the end 10; the other side 13 of the angular reinforcing strip 11 is adherently attached to the edges of the central member through a suitable layer 9 of hardened cement.

In the preparation of the cover portion of the burial vaults of the present invention, the composite sheet 1 of suitable dimensions is bent over a mold 15. The mold 15 may be made of wood and preferably has an arch-shaped form. The wood and sheet material, which is of a plastic puttylike consistency, may be incorporated in a zone having sufficient temperature to accelerate the reaction between the constituents of the cement and to cause hardening in a relatively short time, such as less than five or six hours and preferably less than 1. A temperature of about 125° F. is sufficient to cause hardening in an hour or so and a relatively high humidity is preferred.

Since the magnesium oxychloride cement is of puttylike consistency in the sheets 1, the end portions 10 may be readily cut from such a relatively plastic sheet 1.

The end portions 10 may be hardened separately or preferably may be fastened to the central member 9 prior to the hardening thereof. After hardening of the members 9 and 10, the outer surfaces of the angular reinforcing member 11, which as above set forth is preferably of magnesium oxychloride cement reinforced by fabric material, are coated with magnesium oxychloride cement paste and a member 11 is firmly pressed against each side edge portion of the central member 9 and against the corresponding end 10.

The bottom of the vault consists essentially of a relatively flat central portion 20, which is preferably of rectangular shape to fit into the opening in the lower portion of the cover 6, a peripheral offset portion having a depending portion 21, and a peripheral outwardly extending edge portion 22, upon which the peripheral edges of the cover portion 6 are adapted to rest. The depending portion 21 should be sufficiently high to provide an air seal so that compression of the gases within the chamber of the burial vault will prevent water from rising appreciably above the portion 20. Conventional means (not shown) may be provided for locking the bottom to the cover 6.

The interior as well as the exterior of both the cover and the bottom portion are preferably coated with an adherent layer 16 of asphalt. The outer surface of the vault may have an adherent decorative and waterproofing coating 17. The bottom 20 may be readily formed by deforming one of the sheets 1 of suitable dimensions against a mold of the desired form and allowing the shaped material to set in contact with the mold, preferably at elevated temperatures as above described.

The vaults produced as above described are relatively lightweight, exceedingly strong, and substantially unaffected by moisture or the elements. Since the vaults may be formed from a partially set magnesium cement composition and hardened at elevated temperatures, they are readily adapted for mass production and a large number may be prepared from a relatively small number of molds or forming members.

Although burlap is the preferred fibrous material used for preparing the composite sheet 1, other sheeted fibrous material such as felted or woven fibers, including even tarred paper, may be used if desired.

Although several embodiments of the invention having been herein shown and described, it will be understood that numerous modifications of the construction shown may be resorted to without departing from the spirit of this invention as defined in the appended claims.

What I claim is:

1. In a process of preparing burial vaults from magnesium oxychloride cement compositions, the steps which comprise forming a composite sheet consisting of a plurality of plies of fibrous material, each ply coated with a magnesium oxychloride cement composition of puttylike consistency, shaping said sheet to arch-like form before the hardening of the cement has progressed beyond the stiff puttylike state to provide a central member, preparing cooperating ends from a similar composite sheet material to cooperate with said central member, and adhering the ends to the edges of said central member to obtain a cover member.

2. In a process of preparing burial vaults from magnesium oxychloride cement compositions, the steps which comprise forming a composite sheet consisting of a plurality of plies of fibrous material, each ply coated with a magnesium oxychloride cement composition of puttylike consistency, shaping said sheet to arch-like form before the hardening of the cement has progressed beyond the stiff puttylike state to provide a central member, preparing cooperating ends from a similar composite sheet material to cooperate with said central member, adhering the ends to the edges of said central member to obtain a cover member, forming an angular reinforcing strip from fabric coated with magnesium oxychloride cement of moldable consistency, coating the peripheral adjacent edge portions of said ends and said central member with a layer of magnesium oxychloride cement, disposing said angular reinforcing strip over said coating against said edge portions, and adherently bonding said reinforcing layer to said edge portions through a layer of magnesium oxychloride cement paste.

3. In a process of preparing burial vaults, the steps which comprise coating a fibrous sheet material with magnesium oxychloride cement paste to form coated sheets, superimposing a plurality of said coated sheets with the coatings of adjacent sheets in contact, permitting the magnesium

oxychloride cement thereof to partially set before said magnesium cement composition has set substantially beyond the stiff puttylike consistency to form a composite sheet, forming a composite sheet to generally arch-shape to form a central member, preparing suitable cooperating ends from a similar composite sheet, disposing a plastic material between the peripheral edges of said ends and the edges of said central member, bonding said ends to said central member to form a unitary structure, and allowing the cement composition to harden.

4. In a method of preparing burial vaults, the steps which comprise coating a plurality of sheets of relatively coarsely woven fabric with a magnesium oxychloride cement paste, superimposing a plurality of said coated sheets with the magnesium cement layer of adjacent sheets in contact to form a composite sheet, forming said partially set composite sheet to substantially U-shaped form, allowing the magnesium composition of said shaped composite sheet to harden, preparing suitable end members for cooperation with said shaped composite sheet, and adherently fastening one such end member to said shaped composite sheet at each side edge thereof, whereby a boxlike cover portion of a vault is produced.

5. In a method of preparing burial vaults, the steps which comprise coating a plurality of sheets of relatively coarsely woven fabric with a magnesium oxychloride cement paste, superimposing a plurality of said coated sheets with the magnesium cement layer of adjacent sheets in contact to form a composite sheet, passing said composite sheet into a zone of elevated temperature to accelerate the reaction between the constituents of said magnesium oxychloride cement paste, removing said composite sheet from said zone before the consistency of the magnesium oxychloride cement paste has increased substantially beyond the stiff puttylike state, forming said partially set composite sheet to the form desired for the central member of said vault, allowing the magnesium composition of said shaped composite sheet to harden, preparing suitable end members for cooperation with said shaped composite sheet, and adherently fastening one such end member to said shaped composite sheet at each side edge thereof, whereby a boxlike cover portion of a vault is produced.

6. In a method of preparing burial vaults having a waterproofed surface, the steps which comprise coating a plurality of sheets of relatively coarsely woven fabric with a magnesium oxychloride cement paste, superimposing a plurality of said coated sheets with the magnesium cement layer of adjacent sheets in contact to form a composite sheet, passing said composite sheet into a zone of elevated temperature to accelerate the reaction between the constituents of said magnesium oxychloride cement paste, removing said composite sheet from said zone before the consistency of the magnesium oxychloride cement paste has increased substantially beyond the stiff puttylike state, forming said composite sheet to substantially U-shaped form, disposing said shaped composite sheet in a heated zone to further accelerate the hardening of the cement composition to form a hardened arch-shaped central member, and attaching a suitable cooperating end to each of the side edge portions of said central member to produce a boxlike structure.

7. A burial vault comprising a cover member having an arch-shaped central portion and cooperating end portions attached to said central

portion at the side edge portions thereof, said central portion comprising a shaped composite sheet having a plurality of plies of fabric material, each ply coated with a layer of hardened magnesium oxychloride cement composition, and united to adjacent plies forming a unitary structure.

8. A burial vault comprising a cover member having an arch-shaped central portion and cooperating end portions attached to said central portion at the side edge portions thereof, said central portion being composed essentially of a composite sheet of a plurality of plies of fabric sheet material, each ply coated with a layer of hardened magnesium oxychloride cement composition, the fabric of said outer ply being of relatively finer woven fabric compared to an inner ply, whereby a relatively smooth finish may be had on said central portion.

20 9. In a burial vault having a cover and a cooperating bottom portion, a bottom having a central portion adapted to fit within the opening in the cover member and having a peripheral offset portion with a depending portion and an outwardly extending edge which is adapted to receive said cover member, said central portion and said cooperating ends of said cover member being composed essentially of a plurality of integrally united plies of fabric sheet material, each ply coated with a hardened magnesium oxychloride cement composition.

30 10. In a burial vault having a cover and a cooperating bottom portion, a bottom having a central portion adapted to fit within the opening in the cover member and having a peripheral offset portion with a depending portion and an outwardly extending edge which is adapted to receive said cover member, said central portion and said cooperating ends of said cover member being composed essentially of a plurality of integrally united plies of fabric sheet material, each ply coated with a hardened magnesium oxychloride cement composition, the ply adjacent the outer surface of said central portion and said ends being of finer woven fabric than that of other plies.

35 11. A burial vault comprising a cover member having an arch-shaped central portion, cooperating end portions attached to said central portion at the side edge portions thereof, and a reinforcing strip of angular cross section disposed over the inner edge portions of each end and edge of said central portion and adhered thereto through a layer of hardened plastic material, said central portion being composed essentially of a composite sheet of a plurality of plies of fabric sheet material, each ply coated with a layer of hardened magnesium oxychloride cement composition, the fabric of said outer ply being of relatively finer woven fabric compared to an inner ply, whereby a relatively smooth finish may be had on said central portion.

40 12. In a burial vault having a cover and a cooperating bottom portion, a bottom having a central portion adapted to fit within the opening in the cover member and having a peripheral offset portion with a depending portion and an outwardly extending edge which is adapted to receive said cover member, said cover member and said bottom member being composed of magnesium oxychloride cement composition reinforced with a plurality of plies of sheeted woven fabric material.

45 13. In a burial vault having a cover and a cooperating bottom portion, a bottom having a

central portion adapted to fit within the opening in the cover member and having a peripheral offset portion with a depending portion and an outwardly extending edge which is adapted to receive said cover member, said central portion and said cooperating ends of said cover member being composed essentially of a plurality of integrally united plies of fabric sheet material, each ply coated with a hardened magnesium oxychloride cement composition.

14. In a method of preparing burial vaults, the steps which comprise coating a plurality of sheets of relatively coarsely woven fabric with a magnesium oxychloride cement paste, superimposing a plurality of said coated sheets with the magnesium cement layer of adjacent sheets in contact to form a composite sheet, passing said composite sheet into a suitable zone to permit the reaction between the constituents of said magnesium oxychloride cement paste, removing 20 said composite sheet from said zone before the consistency of the magnesium oxychloride ce-

ment paste has increased substantially beyond the stiff puttylike state, forming said composite sheet to the shape desired for preparing a portion of a boxlike container, and disposing said shaped composite sheet in a heated zone to further accelerate the hardening of the cement composition.

15. A plurality of plies of fabric sheet material adhered together through interposed layers of hardened magnesium oxychloride cement composition, said magnesium cement composition penetrating around and between fibers of said sheet material as when the cement composition is applied in contact with said fibrous sheet material after said fibrous sheet material has been moistened and while said cement composition is in the plastic state, said plies being united together in a unitary structure, being arch-shaped in form and forming a portion of a burial vault.

MAX SKOLNIK.